

April 17, 1951

I. J. HEGYI

2,549,089

MIXED FERRITE COMPOSITIONS, INCLUDING LITHIUM FERRITE

Filed Dec. 15, 1948

2 Sheets-Sheet 1



Fig. 1



Fig. 2  
RESISTIVITIES  
ARE CIRCLED  
 $K = 10^3$  OHMS  
 $M = 10^6$  OHMS

INVENTOR  
IMRE J. HEGYI  
BY  
Moris H. Haskin  
ATTORNEY

April 17, 1951

I. J. HEGYI

2,549,089

MIXED FERRITE COMPOSITIONS, INCLUDING LITHIUM FERRITE

Filed Dec. 15, 1948

2 Sheets-Sheet 2



INVENTOR  
IMRE J. HEGYI  
BY  
Manish Raktin  
ATTORNEY

## UNITED STATES PATENT OFFICE

2,549,089

MIXED FERRITE COMPOSITIONS,  
INCLUDING LITHIUM FERRITEImre J. Hegyi, Princeton, N. J., assignor to Radio  
Corporation of America, a corporation of Dela-  
ware

Application December 15, 1948, Serial No. 65,432

13 Claims. (Cl. 252—62.5)

1

This invention relates to materials having improved magnetic properties. These materials may have unusually high values of magnetic permeability ( $\mu$ ), or they may have desirably low loss values (high Q factor) at radio frequencies, or a usefully high product of these two values.

The materials of the present invention have been found to have unexpectedly high Q values and  $\mu Q$  product at high frequencies (3-30 megacycles). They exhibit unexpectedly high values of D. C. resistance which can be controlled by varying the composition. In addition, they show a desirable reduction in drift compared to most previously known ferrites. (Drift, as used herein, is the term applied to decrease in  $\mu$  with time during the period of measuring the properties of a sample.) They also have unexpectedly higher Curie-temperatures.

More particularly, the invention relates to improved materials of the class known as ferrites. The ferrites are cubic crystalline materials containing  $Fe_2O_3$  and at least one other oxide, usually of a bivalent metal. The ferrites of the present invention may be made by the general method described in the co-pending application of H. W. Leverenz and R. L. Harvey, entitled "Improvement in Magnetic Materials," Serial No. 776,292, filed September 26, 1947.

The present invention relates especially to the incorporation of lithium oxide, an oxide of a monovalent metal, in certain of the ferrite systems previously disclosed.

Whenever "Q" values are mentioned throughout this specification, there is meant a numerical value found by dividing the radio frequency reactance by the resistance of a circuit in which the materials of the present invention are introduced as induction coil core bodies.

By "mixed crystal ferrite" is meant a ferrite material comprising two or more single ferrites which are united in solid solution to form a single homogeneous crystalline material.

One object of the present invention is to provide novel mixed ferrite compositions having improved magnetic properties.

Another object of the invention is to provide novel ferrite materials having controllable and usefully high values of magnetic permeability.

Another object of the invention is to provide novel ferrite materials having unusually high Q factors, especially at relatively high frequencies.

Another object of the invention is to provide novel ferrite materials having unusually high values of  $\mu Q$  product at relatively high frequencies.

2

Another object of the invention is to provide novel ferrite materials having desirable values of resistivity.

Another object of the invention is to provide novel ferrite materials having greatly improved permeability drift characteristics.

Still another object of the present invention is to provide improved ferrite materials having unusually high Curie-temperatures.

These and other objects will be more readily apparent and the invention will be better understood with reference to the following specification, including the drawings of which,

Fig. 1 is a graphical representation illustrating values of  $\mu Q$  product for various compositions in a  $MnO:ZnO:Fe_2O_3$  system with  $LiOH$  added before crystallization at 1000° C. in oxygen, values being measured at 5 megacycles.

Fig. 2 is a plot of the same system and same compositions as shown in Fig. 1 with resistivity and  $\mu$  given for each composition.

Fig. 3 is a plot of the same system as shown in Fig. 1 but with crystallization carried out at 1200° C., and

Fig. 4 is a plot of the same compositions shown in Fig. 3 with values of resistivity and  $\mu$  given for each composition.

Although the compositions which are a part of the present invention are different from those described in the previously mentioned co-pending application, Serial No. 776,292, and also different from those disclosed in co-pending application, Serial No. 795,046, of H. W. Leverenz and I. J. Hegyi, filed December 31, 1947, the general method of preparation is the same as described therein. Optimum heating temperatures and times, however, are not necessarily the same.

Briefly, the general method of preparation of the materials of the present invention includes milling each of the oxide ingredients to a fine state of subdivision, intimately mixing the powdered oxides, preferably forming a compressed body of the mixture, heating the body in an oxidizing atmosphere within a temperature range of about 900° C. to about 1500° C. for from 1 minute to 6 hours, and then cooling. Although rapid cooling is preferred to obtain products with highest permeability, slow cooling may be necessary in some cases to prevent fracture due to the presence of strains. The time of heating will depend upon the size of the body and the temperature, smaller bodies and higher temperatures requiring shorter heating periods. Optimum conditions vary from one composition to another but good results can be obtained with almost any of

the compositions if a heating time of about 1 to 3 hours is used with temperatures of 1000°-1200° C.

The reaction product which is formed in all cases is a composite, homogeneous, crystalline body of cubic structure which does not have the same stoichiometric proportion of oxygen to metals as is present in the mixture before heating, but the exact proportions of the elements, especially oxygen, present in the products is not easily determined.

The oxidizing atmosphere in which the heating of the reaction mixture takes place may be supplied by passing a stream of oxygen through the reaction chamber. Less desirably, air may be used in place of oxygen. It is also possible to form products having improved magnetic permeability and low loss by heating the oxides in a neutral atmosphere, such as one comprising helium or nitrogen, but the improvement is not as great as when an oxidizing atmosphere is used. In general, it may be said that a non-reducing atmosphere is necessary.

Instead of starting with the oxides themselves, it is possible to start with a mixture of metallic compounds which are in other than the oxide form in which they are present in the reaction product, provided these starting materials will be changed to the desired oxide upon heating to the temperatures, times and atmospheric conditions stipulated. For example, instead of starting with a mixture containing  $Fe_2O_3$ , the iron may be in the form of ferrous oxide or the magnetic oxide, provided that heating takes place in an oxidizing atmosphere, and as the hydroxide, carbonate, etc., if either an oxidizing or a neutral atmosphere is present. The other metallic ingredients may also be present initially as hydroxides, carbonates, acetates, etc., if the proper reaction atmosphere is chosen.

Because of the brittleness of the reaction products, compressed bodies of the reactants may be formed at high pressures of, say, 20,000 lbs. per square inch. The compressed bodies may also be formed by extrusion molding processes at much lower pressures. Although, in compression molding, very high pressures are preferred, it has

been found possible to vary the molding pressure widely. Pressures of 2,000 lbs. per square inch have been found to produce the same improved results as pressures ten times as great. Temporary binders may also be used. In general, it has been established that the pressure of forming should be sufficient to form a closely coherent body and the pressure actually chosen may be any one which will produce this result.

10 The reaction mixture may be compressed into any desired shape such as cylindrical or toroidal. Warping may be lessened by mixing a small percentage of a lubricant such as stearic acid or a microcrystalline wax with the ingredients before compressing them. The lubricant should preferably be one which will completely volatilize or burn away during the heating step.

15 The formed bodies are subjected to heat treatment as previously described and then they are cooled. Optimum properties are usually obtained by rapid quenching in air or water but it may be necessary in many cases to cool slowly to avoid the appearance of stresses which will cause fracturing.

20 One important aspect of the present invention is the production of novel ferrite materials comprising various proportions of lithium ferrite, zinc ferrite and manganese ferrite. Table I, below, shows a number of examples of compositions prepared, as above described, by mixing lithium in the form of the hydroxide together with zinc oxide, manganese dioxide and ferric oxide. These compositions, in the form of compressed bodies, were crystallized at 1000° C. in oxygen. Measurements were then made of their magnetic 25 permeability ( $\mu$ ), loss factor (Q) at five megacycles, and D.-C. resistivity in ohms/cm.<sup>3</sup>. The  $\mu Q$  product has also been indicated in each case. Some examples have been included in which no lithium is present, for the sake of illustrating the improvement which occurs when lithium is added. Examples have also been included in which either  $ZnO$  or  $MnO_2$  or both have been omitted, in order to show how the  $\mu Q$  product drops when all three oxides (other than  $Fe_2O_3$ ) are not utilized.

TABLE I

| Code No. | Ingredient Composition |     |                  |                                | Composition for plotting                         |                                    |                                                  | $\mu$ | Q @ 5 Mcs. | $\mu Q$ | d. c. Resistivity, ohms/cm. <sup>3</sup> |
|----------|------------------------|-----|------------------|--------------------------------|--------------------------------------------------|------------------------------------|--------------------------------------------------|-------|------------|---------|------------------------------------------|
|          | LiOH                   | ZnO | MnO <sub>2</sub> | Fe <sub>2</sub> O <sub>3</sub> | MnO <sub>2</sub> .Fe <sub>2</sub> O <sub>3</sub> | ZnO.Fe <sub>2</sub> O <sub>3</sub> | Li <sub>2</sub> O.Fe <sub>2</sub> O <sub>3</sub> |       |            |         |                                          |
| 1316-1   | 0                      | .1  | .9               | 1.0                            | .9                                               | .1                                 | 0                                                | 7.6   | 27         | 205     | 75 K.                                    |
| 1322-1   | .2                     | 0   | .9               | 1.0                            | .9                                               | 0                                  | .1                                               | 24    | 40         | 960     | 2.5 M.                                   |
| 1296-1   | .2                     | .1  | .8               | 1.0                            | .8                                               | .1                                 | .1                                               | 54    | 47         | 2,538   | 1.2 M.                                   |
| 1317-1   | 0                      | .25 | .75              | 1.0                            | .75                                              | .25                                | 0                                                | 22    | 22         | 484     | 0.22 M.                                  |
| 1323-1   | .5                     | 0   | .75              | 1.0                            | .75                                              | 0                                  | .25                                              | 23    | 36         | 828     | 2.0 M.                                   |
| 1299-1   | .1                     | .25 | .7               | 1.0                            | .7                                               | .25                                | .05                                              | 94    | 49         | 4,606   | 1.0 M.                                   |
| 1298-1   | .3                     | .15 | .7               | 1.0                            | .7                                               | .15                                | .15                                              | 70    | 60         | 4,620   | 7.3 M.                                   |
| 1297-1   | .5                     | .05 | .7               | 1.0                            | .7                                               | .05                                | .25                                              | 51    | 35         | 1,785   | 1.8 M.                                   |
| 1324-1   | .8                     | 0   | .6               | 1.0                            | .6                                               | 0                                  | .4                                               | 20    | 35         | 700     | 0.68 M.                                  |
| 1286-2   | .1                     | .35 | .6               | 1.0                            | .6                                               | .35                                | .05                                              | 129   | 39         | 5,031   | 1.1 M.                                   |
| 1287-2   | .3                     | .25 | .6               | 1.0                            | .6                                               | .25                                | .15                                              | 118   | 70         | 8,260   | 1.6 M.                                   |
| 1288-2   | .5                     | .15 | .6               | 1.0                            | .6                                               | .15                                | .25                                              | 98    | 34         | 3,332   | 1.5 M.                                   |
| 1300-1   | .6                     | 0.1 | .6               | 1.0                            | .6                                               | .1                                 | .3                                               | 72    | 30         | 2,160   | 0.73 M.                                  |
| 1318-1   | 0                      | .4  | .6               | 1.0                            | .6                                               | .4                                 | 0                                                | 7.3   | 10         | 73      | 0.6 M.                                   |
| 1301-1   | .1                     | .4  | .55              | 1.0                            | .55                                              | .4                                 | .05                                              | 150   | 53         | 4,800   |                                          |
| 1302-1   | .2                     | .35 | .55              | 1.0                            | .55                                              | .35                                | .1                                               | 167   | 63         | 10,354  | 1.8 M.                                   |
| 1303-1   | .3                     | .3  | .55              | 1.0                            | .55                                              | .3                                 | .15                                              | 147   | 65         | 9,555   | 9.1 M.                                   |
| 1304-1   | .4                     | .25 | .55              | 1.0                            | .55                                              | .25                                | .2                                               | 125   | 52         | 6,500   | 3.6 M.                                   |
| 1319-1   | 0                      | .5  | .5               | 1.0                            | .5                                               | .5                                 | 0                                                | 2.3   | 11         | 25      | 1.1 M.                                   |
| 1305-1   | .1                     | .45 | .5               | 1.0                            | .5                                               | .45                                | .05                                              | 191   | 20         | 3,820   | 1.5 M.                                   |
| 1289-2   | .2                     | .4  | .5               | 1.0                            | .5                                               | .4                                 | .1                                               | 179   | 59         | 10,561  | 4.5 M.                                   |
| 1290-2   | .3                     | .35 | .5               | 1.0                            | .5                                               | .35                                | .15                                              | 169   | 71         | 11,661  | 4.5 M.                                   |
| 1306-1   | .5                     | .3  | .5               | 1.0                            | .5                                               | .3                                 | .2                                               | 143   | 43         | 6,149   |                                          |
| 1291-2   | .5                     | .25 | .5               | 1.0                            | .5                                               | .25                                | .25                                              | 139   | 42         | 5,838   | 5.5 M.                                   |
| 1292-2   | .7                     | .15 | .5               | 1.0                            | .5                                               | .15                                | .35                                              | 58    | 43         | 2,494   | 1.0 M.                                   |
| 1307-1   | .8                     | .1  | .5               | 1.0                            | .5                                               | .1                                 | .4                                               | 28    | 50         | 1,400   |                                          |
| 1325-1   | 1.0                    | 0   | .5               | 1.0                            | .5                                               | 0                                  | .5                                               | 7.3   | 37         | 270     | 2.7 M.                                   |
| 1308-1   | .2                     | .45 | .45              | 1.0                            | .45                                              | .45                                | .1                                               | 174   | 52         | 9,048   | 9.1 M.                                   |
| 1309-1   | .4                     | .35 | .45              | 1.0                            | .45                                              | .3                                 | .2                                               | 191   | 44         | 8,404   | 2.7 M.                                   |

TABLE I—Continued

| Code No. | Ingredient Composition |     |                  |                                | Composition for plotting                         |                                    |                                                  | $\mu$ | Q @ 5 Mcs. | $\mu Q$ | d.c. Resistivity, ohms/cm. <sup>3</sup> |
|----------|------------------------|-----|------------------|--------------------------------|--------------------------------------------------|------------------------------------|--------------------------------------------------|-------|------------|---------|-----------------------------------------|
|          | LiOH                   | ZnO | MnO <sub>2</sub> | Fe <sub>2</sub> O <sub>3</sub> | MnO <sub>2</sub> .Fe <sub>2</sub> O <sub>3</sub> | ZnO.Fe <sub>2</sub> O <sub>3</sub> | Li <sub>2</sub> O.Fe <sub>2</sub> O <sub>3</sub> |       |            |         |                                         |
| 1320-1   | 0                      | .6  | .4               | 1.0                            | .4                                               | .6                                 | 0                                                | 1.3   | 19         | 25      | 1.7 M.                                  |
| 1293-2   | .1                     | .55 | .4               | 1.0                            | .4                                               | .55                                | .05                                              | 149   | 10         | 1,490   | 3.3 M.                                  |
| 1294-2   | .3                     | .45 | .4               | 1.0                            | .4                                               | .45                                | .15                                              | 252   | 30         | 7,560   | 8.2 M.                                  |
| 1295-2   | .5                     | .35 | .4               | 1.0                            | .4                                               | .35                                | .25                                              | 179   | 51         | 9,120   | 1.8 M.                                  |
| 1310-1   | 1.0                    | .1  | .4               | 1.0                            | .4                                               | .1                                 | .5                                               | 23    | 49         | 1,127   | 1.5 M.                                  |
| 1326-1   | 1.2                    | 0   | .4               | 1.0                            | .4                                               | 0                                  | .6                                               | 48    | 34         | 163     | 7.3 M.                                  |
| 1311-1   | .1                     | .6  | .35              | 1.0                            | .35                                              | .6                                 | .05                                              | 141   | 5          | 705     | 3.6 M.                                  |
| 1312-1   | .4                     | .45 | .35              | 1.0                            | .35                                              | .45                                | .2                                               | 265   | 38         | 10,070  | 2.7 M.                                  |
| 1313-1   | .8                     | .25 | .35              | 1.0                            | .35                                              | .25                                | .4                                               | 59    | 62         | 3,658   | 1.4 M.                                  |
| 1314-1   | .3                     | .35 | .3               | 1.0                            | .3                                               | .55                                | .15                                              | 335   | 5          | 1,675   |                                         |
| 1315-1   | .6                     | .4  | .3               | 1.0                            | .3                                               | .4                                 | .3                                               | 140   | 52         | 7,280   | 1.5 M.                                  |
| 1321-1   | 0                      | .75 | .25              | 1.0                            | .25                                              | .75                                | 0                                                | 1.2   | 20         | 24      | 2.9 M.                                  |
| 1327-1   | 1.5                    | 0   | .25              | 1.0                            | .25                                              | 0                                  | .75                                              | 2.8   | 30         | 84      |                                         |
| 1333-1   | .3                     | .65 | .2               | 1.0                            | .2                                               | .65                                | .15                                              | 73    | 3          | 219     | 7.3 M.                                  |
| 1334-1   | .8                     | .4  | .2               | 1.0                            | .2                                               | .4                                 | .4                                               | 46    | 45         | 2,070   | 9.1 M.                                  |
| 1335-1   | 1.3                    | .15 | .2               | 1.0                            | .2                                               | .15                                | .65                                              | 6     | 40         | 240     | 9.1 M.                                  |
| 382-10   | 0                      | 1.0 | 0                | 1.0                            | 0                                                | 1.0                                | 0                                                | 1.01  | 24         | 24      | 90 M.                                   |
| 1328-1   | .5                     | .75 | 0                | 1.0                            | 0                                                | .75                                | .25                                              | 1.03  | 22         | 23      | 18 M.                                   |
| 1329-1   | .8                     | .6  | 0                | 1.0                            | 0                                                | .6                                 | .4                                               | 1.2   | 20         | 24      | 20 M.                                   |
| 1330-1   | 1.0                    | .5  | 0                | 1.0                            | 0                                                | .5                                 | .5                                               | 9     | 15         | 135     | 18 M.                                   |
| 1331-1   | 1.2                    | .4  | 0                | 1.0                            | 0                                                | .4                                 | .6                                               | 5.7   | 27         | 154     | 30 M.                                   |
| 1332-1   | 1.5                    | .25 | 0                | 1.0                            | 0                                                | .25                                | .75                                              | 2.0   | 26         | 52      | 32 M.                                   |
| 1411-10  | 2.0                    | 0   | 0                | 1.0                            | 0                                                | 0                                  | 1.0                                              | 1.01  | 24         | 24      | 3.7 M.                                  |
| 679-10   | 0                      | 0   | 1.0              | 1.0                            | 1.0                                              | 0                                  | 0                                                | 1.01  | 24         | 24      | 1.1 M.                                  |

For resistivity  $K=10^3$  and  $M=10^6$ .

The compositions listed in Table I have been plotted in Fig. 1. For each composition plotted in this figure, the  $\mu Q$  product has also been indicated.

It will be noted that the data given in Table I have been expressed in two different ways. Columns 2, 3, 4 and 5 give the ingredients of each sample in terms of relative number of moles of the compounds which were mixed together. But, in order to simplify the graphical presentation of a quaternary system on a triangular plot, the values given in Columns 2, 3, 4 and 5 have been converted to values which are expressed as relative moles of each corresponding ferrite. These latter values have been listed in Columns 6, 7 and 8 and are assumed to be the approximate proportions of each ferrite present in the final product.

Complete data, from which the examples listed in Table I have been chosen, show that useful improvements in  $\mu Q$  product are obtained when compositions are made up comprising about 0.01 to about 32.5 mole per cent Li<sub>2</sub>O, about 2.5 to about 30 mole per cent ZnO and about 10 to about 42.5 mole per cent MnO<sub>2</sub>. Although all of the tabulated examples are directed to compositions containing 50 mole per cent Fe<sub>2</sub>O<sub>3</sub> for the sake of comparison, experiment has shown that the Fe<sub>2</sub>O<sub>3</sub> content may be varied between about 30 and about 70 mole per cent.

From an inspection of the values of  $\mu Q$  product plotted on Fig. 1, an area will be noted in which the values are exceptionally high. This area may be defined by the range of compositions in which there are present Fe<sub>2</sub>O<sub>3</sub>—50 mole per cent, Li<sub>2</sub>O—2.5 to 12.5 mole per cent, MnO<sub>2</sub>—15 to 35 mole per cent and at least one oxide from the class consisting of ZnO and CdO—10 to 25 mole per cent. This is to be taken as the preferred range of compositions. Preferred time of heating at this temperature is 3 hours, although it may be from 1 minute to 6 hours. These values are found at relatively high frequencies of 3-30 megacycles.

Within the preferred range an optimum composition is found comprising Fe<sub>2</sub>O<sub>3</sub>—50 mole per cent, MnO<sub>2</sub>—25 mole per cent, ZnO (or CdO, or both together)—17.5 mole per cent and Li<sub>2</sub>O—7.5 mole per cent. On Fig. 1, this composition

corresponds to a product having the proportions MnO<sub>2</sub>.Fe<sub>2</sub>O<sub>3</sub>—50 mole per cent, ZnO.Fe<sub>2</sub>O<sub>3</sub>—35 mole per cent and Li<sub>2</sub>O.Fe<sub>2</sub>O<sub>3</sub>—15 mole per cent.

The best range of compositions to produce products having highest resistivities and useful values of  $\mu$  is Fe<sub>2</sub>O<sub>3</sub>—50 mole per cent, MnO<sub>2</sub>—15 to 35 mole per cent, ZnO (or CdO, or both together)—7.5 to 32.5 mole per cent and Li<sub>2</sub>O—2.5 to 12.5 mole per cent. On Fig. 1, this corresponds to a product composition of MnO<sub>2</sub>—30 to 70 mole per cent, ZnO.Fe<sub>2</sub>O<sub>3</sub>—15 to 65 mole per cent and Li<sub>2</sub>O.Fe<sub>2</sub>O<sub>3</sub>—5 to 25 mole per cent. Crystallization should take place at 950-1250° C. and the preferred time is about 1 1/2 hours, although this may also range from 1 minute to 6 hours.

Fig. 2 is a plot of most of the same compositions shown in Fig. 1 but, in this case, the resistivity and permeability values are given for each composition. The values in this figure show that the D.-C. resistivity of the materials can be controlled by varying the Li<sub>2</sub>O content of the reaction mixture. Materials having high D.-C. resistivity are useful in various types of apparatus. For example, in some applications, two or more coils are wound on the same ferrite, with one coil having a higher D.-C. voltage than the other. In such a case, to be able to wind the coil directly upon the ferrite without the addition of an insulator between the ferrite and the coil, the ferrite must have high resistivity. Also, when a ferrite core must be mounted directly upon a chassis, it is advantageous that it have a high resistivity.

In the above described ferrite system, it is possible to substitute CdO for some or all of the ZnO and obtain materials having unusually high values of magnetic permeability, high Q factor and high D.-C. resistivity. Table II shows some examples of this type of composition and measured values of  $\mu$ , Q at 5 megacycles and D.-C. resistivity. In some instances, the ZnO was completely replaced by CdO, while in other examples the compositions contained both ZnO and CdO. It has been concluded from a more complete set of measurements that the compositions may contain the same mole percentages of CdO as found for ZnO or that the percentage given for ZnO may be divided in any ratio between CdO and ZnO.

TABLE II  
[Crystallized at 1000° C. in oxygen.]

| Code No. | ZnO <sub>0.5</sub> Fe <sub>2</sub> O <sub>3</sub> | CdO <sub>0.5</sub> Fe <sub>2</sub> O <sub>3</sub> | Li <sub>2</sub> O <sub>0.5</sub> Fe <sub>2</sub> O <sub>3</sub> | MnO <sub>0.5</sub> Fe <sub>2</sub> O <sub>3</sub> | $\mu$ | Q @ 5 mcs. | $\mu Q$ | D. C. Resistivity, ohms/cm. <sup>3</sup> |
|----------|---------------------------------------------------|---------------------------------------------------|-----------------------------------------------------------------|---------------------------------------------------|-------|------------|---------|------------------------------------------|
| 1517-3   | 0                                                 | 0.5                                               | 0                                                               | 0.5                                               | 1.4   | 18         | 25      | 470 K.                                   |
| 1518-3   | 0                                                 | 0.4                                               | 0.1                                                             | 0.5                                               | 292   | 17         | 5,264   | 360 K.                                   |
| 1519-3   | 0                                                 | 0.35                                              | 0.15                                                            | 0.5                                               | 262   | 34         | 8,909   | 5 M.                                     |
| 1520-3   | 0                                                 | 0.3                                               | 0.2                                                             | 0.5                                               | 198   | 40         | 7,920   | 11 M.                                    |
| 1521-3   | 0.1                                               | 0.25                                              | 0.15                                                            | 0.5                                               | 230   | 42         | 9,660   | 18 M.                                    |
| 1522-3   | 0.175                                             | 0.175                                             | 0.15                                                            | 0.5                                               | 234   | 48         | 11,232  | 9 M.                                     |
| 1523-3   | 0.25                                              | 0.1                                               | 0.15                                                            | 0.5                                               | 230   | 52         | 11,960  | 22 M.                                    |

Table III gives a number of examples of the same ferrite system MnO:ZnO (or CdO, or ZnO and CdO): Li<sub>2</sub>O:Fe<sub>2</sub>O<sub>3</sub> with crystallization being

and 4, Figure 3 giving the  $\mu Q$  product of each composition and Figure 4 giving the D.-C. resistivity and permeability values.

TABLE III  
MnO:ZnO:Fe<sub>2</sub>O<sub>3</sub> system with LiOH addition (before crystallization at 1200° C. in oxygen)

| Code No. | MnO <sub>0.5</sub> Fe <sub>2</sub> O <sub>3</sub> | ZnO <sub>0.5</sub> Fe <sub>2</sub> O <sub>3</sub> | Li <sub>2</sub> O <sub>0.5</sub> Fe <sub>2</sub> O <sub>3</sub> | $\mu$ | Q @ 5 mcs. | $\mu Q$ | D. C. Resistivity, ohms/cm. <sup>3</sup> |
|----------|---------------------------------------------------|---------------------------------------------------|-----------------------------------------------------------------|-------|------------|---------|------------------------------------------|
| 1316-3   | .9                                                | .1                                                | 0                                                               | 338   | 5          | 1,690   | 1.12 K.                                  |
| 1296-3   | .8                                                | .1                                                | .1                                                              | 146   | 15         | 2,390   | 0.23 M.                                  |
| 1317-3   | .75                                               | .25                                               | 0                                                               | 463   | 3          | 1,389   | 1.0 K.                                   |
| 1322-3   | .75                                               | 0                                                 | .25                                                             | 76    | 23         | 1,748   | 6.9 M.                                   |
| 1297-3   | .7                                                | .05                                               | .25                                                             | 82    | 25         | 2,050   | 3.8 M.                                   |
| 1298-3   | .7                                                | .15                                               | .15                                                             | 155   | 20         | 3,100   | 0.75 M.                                  |
| 1299-3   | .7                                                | .25                                               | .05                                                             | 318   | 5          | 1,590   | 22 K.                                    |
| 1318-3   | .6                                                | .4                                                | 0                                                               | 530   | 3          | 1,590   | 280.                                     |
| 1286-3   | .6                                                | .35                                               | .05                                                             | 373   | 5          | 1,863   | 19.5 K.                                  |
| 1287-3   | .6                                                | .25                                               | .15                                                             | 202   | 20         | 4,040   | 1.3 M.                                   |
| 1288-3   | .6                                                | .15                                               | .25                                                             | 112   | 27         | 3,024   | 5.5 M.                                   |
| 1300-3   | .6                                                | .1                                                | .3                                                              | 91    | 27         | 2,457   | 4.5 M.                                   |
| 1324-3   | .6                                                | 0                                                 | .4                                                              | 36    | 25         | 900     | 3.6 M.                                   |
| 1301-3   | .55                                               | .4                                                | .05                                                             | 404   | 5          | 2,020   | 20 K.                                    |
| 1302-3   | .55                                               | .35                                               | .10                                                             | 313   | 11         | 3,443   | 0.19 M.                                  |
| 1303-3   | .55                                               | .30                                               | .15                                                             | 228   | 22         | 5,016   | 2.7 M.                                   |
| 1304-3   | .55                                               | .25                                               | .20                                                             | 190   | 28         | 5,320   | 4.0 M.                                   |
| 1319-3   | .5                                                | .5                                                | 0                                                               | 540   | 3          | 1,620   | 310.                                     |
| 1305-3   | .5                                                | .45                                               | .05                                                             | 407   | 5          | 2,035   | 28 K.                                    |
| 1289-3   | .5                                                | .4                                                | .1                                                              | 322   | 10         | 3,220   | 250 K.                                   |
| 1290-3   | .5                                                | .35                                               | .15                                                             | 262   | 19         | 4,978   | 1.3 M.                                   |
| 1291-3   | .5                                                | .25                                               | .25                                                             | ----- | -----      | -----   | 0.73 M.                                  |
| 1292-3   | .5                                                | .15                                               | .35                                                             | ----- | -----      | -----   | 3.6 M.                                   |
| 1325-3   | .5                                                | 0                                                 | .5                                                              | 19    | 27         | 513     | 3.6 M.                                   |
| 1308-3   | .45                                               | .45                                               | .1                                                              | 342   | 5          | 1,710   | -----                                    |
| 1309-3   | .45                                               | .3                                                | .2                                                              | 232   | 22         | 5,104   | 7.3 M.                                   |
| 1320-3   | .4                                                | .6                                                | 0                                                               | 33    | 2          | 66      | 210.                                     |
| 1293-3   | .4                                                | .55                                               | .05                                                             | ----- | -----      | -----   | 31 K.                                    |
| 1294-3   | .4                                                | .45                                               | .15                                                             | 328   | 5          | 1,640   | 4.0 M.                                   |
| 1295-3   | .4                                                | .35                                               | .25                                                             | 192   | 18         | 3,456   | 3.3 M.                                   |
| 1310-3   | .4                                                | .1                                                | .5                                                              | 21    | 36         | 756     | 8.2 M.                                   |
| 1326-3   | .4                                                | 0                                                 | .6                                                              | 10    | 25         | 250     | 4.5 M.                                   |
| 1311-3   | .35                                               | .6                                                | .05                                                             | 488   | 5          | 2,440   | 22 K.                                    |
| 1312-3   | .35                                               | .45                                               | .2                                                              | 277   | 5          | 1,385   | 4.5 M.                                   |
| 1313-3   | .35                                               | .25                                               | .4                                                              | 61    | 31         | 1,891   | 5.5 M.                                   |
| 1314-3   | .3                                                | .55                                               | .15                                                             | 427   | 2          | 854     | 4.0 M.                                   |
| 1315-3   | .3                                                | .4                                                | .3                                                              | 169   | 10         | 1,690   | 3.8 M.                                   |
| 1321-3   | .25                                               | .75                                               | 0                                                               | 1.1   | 22         | 24      | 230.                                     |
| 1327-3   | .25                                               | 0                                                 | .75                                                             | 6     | 20         | 120     | -----                                    |
| 1333-3   | .2                                                | .65                                               | .15                                                             | 175   | 3          | 525     | 8.2 M.                                   |
| 1334-3   | .2                                                | .4                                                | .4                                                              | 89    | 5          | 440     | 0.79 M.                                  |
| 1335-3   | .2                                                | .15                                               | .65                                                             | 11    | 25         | 275     | 7.3 M.                                   |
| 1328-3   | 0                                                 | .75                                               | .25                                                             | 1.2   | 21         | 25      | 120.                                     |
| 1329-3   | 0                                                 | .6                                                | .4                                                              | 39    | 2          | 78      | 190.                                     |
| 1330-3   | 0                                                 | .5                                                | .5                                                              | 32    | 3          | 98      | 260.                                     |
| 1331-3   | 0                                                 | .4                                                | .6                                                              | 15    | 5          | 75      | -----                                    |
| 1332-3   | 0                                                 | .25                                               | .75                                                             | 5     | 18         | 90      | -----                                    |
| 352-12   | 0                                                 | 1.0                                               | 0                                                               | 1.02  | 22         | 22      | 590.                                     |
| 1411-12  | 0                                                 | 0                                                 | 1.0                                                             | 1.14  | 22         | 24      | 204 K.                                   |
| 679-12   | 1.0                                               | 0                                                 | 0                                                               | 216   | 10         | 2,160   | 12.4 K.                                  |

carried out at 1200° C. in oxygen. Although the  $\mu Q$  product is different and, in general, somewhat lower, in each case, than for the same compositions crystallized at 1000° C., the range of percentages producing useful products is substantially the same as previously given. The data given in this table are plotted in Figures 3

Table IV is the corresponding table for compositions containing CdO either partially or wholly substituted for ZnO. As in the case of compositions prepared at 1000° C., it has been found that when prepared by heating at 1200° C., cadmium oxide may be substituted for zinc oxide either partially or totally and in any ratio.

TABLE IV  
[Crystallized at 1200° C. in oxygen.]

| Code No. | ZnO <sub>0.5</sub> Fe <sub>2</sub> O <sub>3</sub> | CdO <sub>0.5</sub> Fe <sub>2</sub> O <sub>3</sub> | Li <sub>2</sub> O <sub>0.5</sub> Fe <sub>2</sub> O <sub>3</sub> | MnO <sub>0.5</sub> Fe <sub>2</sub> O | $\mu$ | Q @ 5 mcs. | $\mu Q$ | D. C. Resistivity ohms/cm. <sup>3</sup> |
|----------|---------------------------------------------------|---------------------------------------------------|-----------------------------------------------------------------|--------------------------------------|-------|------------|---------|-----------------------------------------|
| 1517-1   | 0                                                 | 0.5                                               | 0                                                               | 0.5                                  | 540   | 2          | 1,080   | 150.                                    |
| 1518-1   | 0                                                 | 0.4                                               | 0.1                                                             | 0.5                                  | 338   | 3          | 999     | 34 K.                                   |
| 1519-1   | 0                                                 | 0.35                                              | 0.15                                                            | 0.5                                  | 245   | 18         | 3,610   | 580 K.                                  |
| 1520-1   | 0                                                 | 0.3                                               | 0.2                                                             | 0.5                                  | 203   | 23         | 4,669   | 1.3 M.                                  |
| 1521-1   | 0.1                                               | 0.25                                              | 0.15                                                            | 0.5                                  | 242   | 20         | 4,840   | 1.3 M.                                  |
| 1522-1   | 0.175                                             | 0.175                                             | 0.15                                                            | 0.5                                  | 245   | 23         | 5,635   | 1.8 M.                                  |
| 1523-1   | 0.25                                              | 0.1                                               | 0.5                                                             | 0.5                                  | 251   | 25         | 6,275   | 3.3 M.                                  |

TABLE VII

*BeO:ZnO:MnO:Fe<sub>2</sub>O<sub>3</sub> with LiOH addition (before crystallization at 1200° C. in oxygen)*

| Code No. | LiOH | BeO  | ZnO  | MnO <sub>2</sub> | Fe <sub>2</sub> O <sub>3</sub> | $\mu$ | Q @ 1/2 mcs. | $\mu Q$ | $\Delta\mu$ in 2 minutes |
|----------|------|------|------|------------------|--------------------------------|-------|--------------|---------|--------------------------|
| 1003-1   | 0    | .05  | .20  | .25              | .5                             | 416   | 78           | 32,458  | Per cent                 |
| 1008-1   | .02  | .05  | .20  | .25              | .5                             | 441   | 73           | 32,193  | -1.1                     |
| 1009-1   | .04  | .05  | .20  | .25              | .5                             | 463   | 70           | 32,410  | -0.6                     |
| 1010-1   | .08  | .05  | .20  | .25              | .5                             | 441   | 80           | 35,280  | -0.6                     |
| 1015-1   | 0    | .075 | .175 | .25              | .5                             | 393   | 85           | 35,405  | -1.5                     |
| 1020-1   | .02  | .075 | .175 | .25              | .5                             | 396   | 82           | 34,472  | -1.1                     |
| 1021-1   | .04  | .075 | .175 | .25              | .5                             | 413   | 78           | 33,014  | -0.9                     |
| 1022-1   | .08  | .075 | .175 | .25              | .5                             | 396   | 96           | 35,016  | -0.2                     |

Another category in which unexpected improvement has been found by adding Li<sub>2</sub>O·Fe<sub>2</sub>O<sub>3</sub> to the MnO·Fe<sub>2</sub>O<sub>3</sub>·ZnO·Fe<sub>2</sub>O<sub>3</sub> system is that of controlling the Curie-temperature of the product. The Curie-temperature is the temperature at which the initial permeability has fallen to a slight fraction of approximately 10% of the maximum value. It is of great advantage that the Curie-temperature of any of the ferrites which are to be used as core materials be far above room or other ordinary operating temperature so that a change in temperature will not cause a relatively large change in permeability.

Table VIII, below, shows the Curie-temperatures of a number of examples of ferrites in the system MnO·Fe<sub>2</sub>O<sub>3</sub>·ZnO·Fe<sub>2</sub>O<sub>3</sub>·Li<sub>2</sub>O·Fe<sub>2</sub>O<sub>3</sub>.

usually an optimum heating temperature, however, for each composition.

I claim as my invention:

1. A cubic crystalline ferrite material consisting essentially of the reaction product produced by heating together in a non-reducing atmosphere at temperatures of from about 900° C. to about 1500° C. for from about 1 minute to about 6 hours an intimate mixture of about 30 to about 70 mole per cent Fe<sub>2</sub>O<sub>3</sub>, about 0.01 to about 32.5 mole per cent Li<sub>2</sub>O, about 2.5 to about 30 mole per cent of at least one oxide from the class consisting of ZnO and CdO and about 10 to about 42.5 mole per cent of MnO<sub>2</sub>.

2. A ferrite material according to claim 1 in which said heating temperature is from 1000°

TABLE VIII

| Code No. | MnO·Fe <sub>2</sub> O <sub>3</sub> | ZnO·Fe <sub>2</sub> O <sub>3</sub> | Li <sub>2</sub> O·Fe <sub>2</sub> O <sub>3</sub> | Crystallization Temperature | Curie-Temperature |
|----------|------------------------------------|------------------------------------|--------------------------------------------------|-----------------------------|-------------------|
| 1312-1   | .35                                | .45                                | .2                                               | 1000                        | 280               |
| 1293-1   | .4                                 | .55                                | .05                                              | 1000                        | 145               |
| 1294-2   | .4                                 | .45                                | .15                                              | 1000                        | 283               |
| 679-1    | .5                                 | .5                                 | 0                                                | 1200                        | 280               |
| 1305-1   | .5                                 | .45                                | .05                                              | 1000                        | 185               |
| 1289-2   | .5                                 | .4                                 | .1                                               | 1000                        | 280               |
| 1290-2   | .5                                 | .35                                | .15                                              | 1000                        | 342               |
| 1306-1   | .5                                 | .3                                 | .2                                               | 1000                        | 358               |
| 1318-3   | .6                                 | .4                                 | 0                                                | 1200                        | 217               |
| 1286-2   | .6                                 | .35                                | .05                                              | 1000                        | 210               |
| 1287-2   | .6                                 | .25                                | .15                                              | 1000                        | 375               |
| 1299-1   | .7                                 | .25                                | .05                                              | 1000                        | 261               |
| 1298-1   | .7                                 | .15                                | .16                                              | 1000                        | 410               |

These examples show that the Curie-temperature is raised when Li<sub>2</sub>O·Fe<sub>2</sub>O<sub>3</sub> is added to the Mn-Zn ferrite system. Although only a few examples out of a large number have been tabulated, complete data indicate that a rise in Curie-temperature is obtained by adding the same proportions of Li<sub>2</sub>O and using the same proportions of the other ingredients set forth in the previous definition of the limits of the compositions.

There have thus been described improved ferrite materials exhibiting unexpected improvements in several of their useful magnetic properties. The proportions of the ingredients used should, in general, be within the percentage ranges given since use of other proportions results in products which either are not significantly improved or are inferior to previously known ferrites.

A range of time and temperature of heating has also been given. The size of the body influences the time necessary to bring about a complete reaction of the oxides. Very small bodies require much shorter heating times than large bodies. Also, the required time of heating is usually in inverse ratio to the temperature used. There is

1200° C.

3. A ferrite material according to claim 2 in which said atmosphere is an oxidizing atmosphere.

4. A ferrite material according to claim 1 in which the reaction mixture includes also from about 0.2 to about 50 mole per cent BeO.

5. A ferrite composition according to claim 1 in which said heating temperature is 1000° C. and the ingredients of the reaction mixture are present in the following proportions: Fe<sub>2</sub>O<sub>3</sub>—50 mole per cent, Li<sub>2</sub>O—2.5 to 12.5 mole per cent, MnO<sub>2</sub>—15 to 35 mole per cent and at least one oxide from the class consisting of ZnO and CdO—10 to 25 mole per cent.

6. An article of manufacture characterized by having a relatively high value of  $\mu Q$  product, said article being a compressed body of material having a predetermined shape, said material consisting essentially of a reaction product produced by heating together at temperatures of 900°-1500° C. for from 1 minute to 6 hours in a non-reducing atmosphere an intimate mixture of about 30 to about 70 mole per cent Fe<sub>2</sub>O<sub>3</sub>, about 0.01 to about 32.5 per cent Li<sub>2</sub>O,

A study of the above given data leads one to the conclusion that, if LiOH is not added to these ferrite systems, the optimum permeability ( $\mu$ ) is

MnO<sub>2</sub> and Fe<sub>2</sub>O<sub>3</sub>. CdO can be substituted for part or all of the ZnO. In these examples, crystallization was carried out at 1200° C. in oxygen.

TABLE V  
*BeO:ZnO:MnO<sub>2</sub>:Fe<sub>2</sub>O<sub>3</sub> with LiOH addition (before crystallization at 1200° C. in oxygen)*

| Code No. | LiOH | BeO  | ZnO  | MnO <sub>2</sub> | Fe <sub>2</sub> O <sub>3</sub> | $\mu$ | Q @ 5 mcs. | $\mu Q$ | D. C. Resistivity, ohms/cm. <sup>2</sup> |
|----------|------|------|------|------------------|--------------------------------|-------|------------|---------|------------------------------------------|
| 485-12   | 0    | .075 | .175 | .25              | .5                             | 430   | 4          | 1,720   | 70.                                      |
| 1423-12  | .05  | .075 | .175 | .25              | .5                             | 413   | 5          | 2,065   | 1.6 K.                                   |
| 1424-12  | .1   | .075 | .175 | .25              | .5                             | 316   | 10         | 3,160   | 185 K.                                   |
| 1426-12  | .2   | .075 | .175 | .25              | .5                             | 223   | 25         | 5,575   | 6.7 M.                                   |

obtained using a crystallization temperature of 1200° C. However, when LiOH is added, optimum  $\mu Q$  products are produced using a crystallization temperature of 1000° C. Higher  $\mu Q$  products are observed even though the value of  $\mu$  drops somewhat with increasing amounts of LiOH added to the composition, for the value of Q rises rapidly enough to more than compensate for the diminishing value of  $\mu$ .

In some uses, however, the Q factor of a material may not be as important as its magnetic permeability or its D.-C. resistivity. For such uses, the preferred type of composition in the system of this aspect of the present invention would be that in which crystallization is carried out at 1200° C. since higher values of both  $\mu$  and D.-C.

Although only a few selected examples have been given in the above table, more complete data indicate that lithium may be present as Li<sub>2</sub>O in the proportion of about .01 to about 32.5 mole per cent, BeO may be used in the proportion of about 0.2 to about 50 mole per cent, Fe<sub>2</sub>O<sub>3</sub> may be present in the proportion of about 30 to about 70 mole per cent and the remainder may be either ZnO, CdO or any ratio of both. In general, the proportions (for all except Li<sub>2</sub>O) are the same as those disclosed in the above mentioned co-pending application, Serial No. 795,046.

Table VI gives examples of ferrites prepared from the same materials as given in Table V but crystallized at 1100° C. in oxygen.

TABLE VI  
*BeO:ZnO:MnO<sub>2</sub>:Fe<sub>2</sub>O<sub>3</sub> with LiOH addition (before crystallization at 1100° C. in oxygen)*

| Code No. | LiOH | BeO  | ZnO | MnO <sub>2</sub> | Fe <sub>2</sub> O <sub>3</sub> | $\mu$ | Q @ 5 mcs. | $\mu Q$ | D. C. Resistivity, ohms/cm. <sup>2</sup> |
|----------|------|------|-----|------------------|--------------------------------|-------|------------|---------|------------------------------------------|
| 482      | 0    | .05  | .20 | .25              | .5                             | 180   | 2          | 360     |                                          |
| 1266-2   | .025 | .025 | .20 | .25              | .5                             | 264   | 7          | 1,348   | 62.7 K.                                  |
| 1267-2   | .05  | .025 | .20 | .25              | .5                             | 343   | 17         | 5,331   | 91 K.                                    |
| 486      | 0    | .10  | .15 | .25              | .5                             | 91    | 2          | 182     |                                          |
| 1270-2   | .05  | .05  | .15 | .25              | .5                             | 223   | 26         | 5,798   | 52.8 K.                                  |
| 1271-2   | .1   | .05  | .15 | .25              | .5                             | 235   | 37         | 8,695   | 291 K.                                   |
| 1412     | 0    | .15  | .1  | .25              | .5                             | 27    | 30         | 810     |                                          |
| 1272-2   | .05  | .1   | .25 | .5               | 108                            | 34    | 3,672      | 63.5 K. |                                          |
| 1273-2   | .1   | .05  | .1  | .25              | .5                             | 156   | 36         | 5,610   | 106 K.                                   |
| 0275-2   | .2   | .05  | .1  | .25              | .5                             | 143   | 45         | 6,435   | 6.26 M.                                  |

resistivity may be obtained using this temperature.

It is also evident, from a study of the above given data, that, by adding LiOH (or its equivalent amount of Li<sub>2</sub>O) to the given ferrite material pre-mix, there can be obtained a magnetic material with controllable and higher Q factor and  $\mu Q$  product and also a material having controllable and higher D.-C. resistivity. In these respects, materials are produced which are unexpectedly superior to manganese ferrites, manganese-zinc ferrites, lithium ferrites or lithium-zinc ferrites.

In another co-pending application of H. W. Leverenz and I. J. Hegyi, Serial No. 795,046, filed December 31, 1947, there have been disclosed ferrite compositions made from beryllium oxide in addition to zinc oxide and/or cadmium oxide, and manganese oxide. It has now been found that, when LiOH is added to these compositions, materials are produced having improved  $\mu Q$  products and higher D.-C. resistivities. Table V, below, gives a few examples of ferrite compositions made from various mixtures of LiOH, BeO, ZnO,

55 The above examples show that when LiOH (or the equivalent amount of Li<sub>2</sub>O) is added to the system BeO:ZnO:MnO<sub>2</sub>:Fe<sub>2</sub>O<sub>3</sub>, a controllable increase in  $\mu Q$  product may be obtained in the crystalline ferrite which is produced. CdO may, as before, be substituted for part or all of the ZnO.

Many of the previously prepared ferrites exhibit an instability of certain of their magnetic properties which greatly detracts from their usefulness. For example, they often exhibit a phenomenon known as "drift" which is the term applied to a decrease in  $\mu$  which occurs over the period of time that the magnetic permeability is being measured. "Drift" is usually more pronounced at lower frequencies of, say, the order of 0.5 megacycle. It has been found that when lithium ferrite is added to certain of the ferrites which exhibit "drift" the "drift" is decreased. Examples of this property are shown in Table VII, below, for systems of crystalline ferrites made up by adding LiOH to mixtures of BeO:ZnO (or CdO, or both ZnO and CdO):MnO<sub>2</sub>:Fe<sub>2</sub>O<sub>3</sub>. Crystallization was at 1200° C. in oxygen.

about 2.5 to about 30 mole per cent of at least one oxide from the class consisting of  $ZnO$  and  $CdO$ , and about 10 to about 42.5 mole per cent  $MnO_2$ .

7. An article according to claim 6 in which said temperatures are  $1000^{\circ}$ – $1200^{\circ}$  C.

8. An article according to claim 7 in which said atmosphere is an oxidizing atmosphere.

9. A method of forming a core body having a relatively high value of  $\mu Q$  product comprising preparing an intimate mixture consisting essentially of stoichiometric proportions of  $Fe_2O_3$ ,  $Li_2O$ ,  $MnO_2$  and at least one oxide from the class consisting of  $ZnO$  and  $CdO$ , compressing said mixture to form a coherent molded body of predetermined shape, subjecting said molded body to a temperature of  $900^{\circ}$ – $1500^{\circ}$  C. in an oxidizing atmosphere to form a homogeneous cubic crystalline ferrite material and cooling said body.

10. A method of raising the Curie-temperature of a cubic crystalline ferrite body consisting essentially of manganese ferrite and at least one of a class consisting of zinc ferrite and cadmium ferrite, comprising incorporating therewith from 0.02 to 65 mole per cent of lithium ferrite.

11. A homogeneous cubic crystalline ferrite body consisting essentially of about 0.02 to about

65 mole per cent lithium ferrite, about 5 to about 60 mole per cent of a ferrite from the class consisting of cadmium ferrite and zinc ferrite and about 20 to about 85 mole per cent manganese ferrite.

5 12. A homogeneous cubic crystalline ferrite body having relatively high  $\mu Q$  product at 3–30 megacycles consisting essentially of about 50 mole per cent  $MnO.Fe_2O_3$ , 35 mole per cent  $ZnO.Fe_2O_3$  and 15 mole per cent  $Li_2O.Fe_2O_3$ .

10 13. A homogeneous cubic crystalline ferrite body having relatively high resistivity consisting essentially of the reaction product produced by heating together at  $950$ – $1250^{\circ}$  C. for from 1 minute to 6 hours in an oxidizing atmosphere  $Fe_2O_3$ —50 mole per cent,  $MnO_2$ —15 to 35 mole per cent, at least one oxide from the class consisting of  $ZnO$  and  $CdO$ —7.5 to 32.5 mole per cent and  $Li_2O$ —2.5 to 12.5 mole per cent.

20 IMRE J. HEGYI.

#### REFERENCES CITED

The following references are of record in the file of this patent:

25 Kawai, Journal of the Society of Chemical Industry, Japan, vol. 37, No 4, 1934; page 174B.